

# UNITED STATES PATENT OFFICE.

ALEXANDRE WAGANOFF, OF PETROGRAD, RUSSIA.

## TREATMENT OF THE BAST OF THE LINDEN OR LIME-TREE AND WILLOW FOR THE MANUFACTURE OF WEBS.

1,149,876.

Specification of Letters Patent. Patented Aug. 10, 1915.

No Drawing.

Application filed February 6, 1915. Serial No. 6,633.

To all whom it may concern:

Be it known that I, ALEXANDRE WAGANOFF, a subject of the Emperor of Russia, residing at Kamennoostrowski Perspective, 5 house 24, Petrograd, Russia, have invented certain new and useful Improvements in the Treatment of the Bast of the Linden or Lime-Tree and Willow for the Manufacture of Webs; and I do hereby declare the following to be a full, clear, and exact description of the invention, such as will enable others skilled in the art to which it appertains to make and use the same.

The fibers of the linden or lime-tree and 15 those of the willow are distinguished, as is well known, by a great strength against stretching forces. Nevertheless the said fibrous material has been used up to the present only for the manufacture of 20 matting and like webs in which the woof and warp have but a very small length.

The object of this invention is to produce from the bast of the linden or lime-tree and the willow long threads which may 25 be used on a loom in the ordinary way for the manufacture of webs of various kinds. To that effect the films of bast or inner bark of the said trees, separated from the outer bark, are boiled in an open or tightly 30 closed vessel with an alkaline liquid to make the same soft and capable to be subdivided in the longitudinal direction. The concentration of the alkaline liquid and the duration of the said boiling process depend 35 upon the origin of the bast. The bast received from an old tree f. i. must be boiled a longer time than that from a young tree. If the boiling is effected in an open receptacle the same takes about two hours. The 40 bast films softened in the manner just described are then placed upon a table end-by-end and cemented together using pasted paper strips or the like, which are stucked to the adjacent ends of the strips on both 45 or only on the one side. The long bast-film thus produced is then subdivided, by means of appropriate devices, into long narrow strips or flat threads which are then spooled and finally used on looms in the ordinary 50 way.

The dividing of the bast-films into flat threads may be attained f. i. by passing the films between a flat and a ribbed cylinder or by means of edged rotating disks.

55 If it is desired to produce from the bast

fine webs, the bast-films are submitted, after the first boiling, to a second boiling process effected during 15-30 minutes within a closed vessel containing a 2%-3% liquid of soluble glass with a view to receive a fibrous 60 material which can be without any difficulties decomposed into primary fibrils and then spun to threads either separately or in combination with fibrils of another origin, as f. i. hemp, lime, etc. Such fibrils of another origin may be also brought into the webs produced from the flat or spun threads of bast by using the threads of bast and the threads from another fibrous material 65 conjointly and alternately in separate shuttles 70 of one and the same loom. In such way webs of very various qualities may be manufactured, which webs or textures may be submitted to all the known treatments with a view to change the aspect or color of their 75 surface or to render same waterproof.

What I claim is:

1. Improvements in the treatment of the bast of the linden or lime-tree and willow for the manufacture of webs, consisting in 80 boiling the bast separated from the outer bark within an alkaline liquid, cementing together the ends of the separate short bast-films to form a long film, subdividing the latter into strips or flat threads, spooling the 85 said strips or threads and utilizing the same in the shuttles of ordinary looms.

2. Improvements in the treatment of the bast of the linden or lime-tree and willow for the manufacture of webs, consisting in 90 boiling the bast in an alkaline liquid, submitting the same to a second boiling process during 15-30 minutes within a closed vessel containing a 2%-3% liquid of soluble glass, subdividing the softened bast into elementary fibrils, spinning threads from said fibrils and using the threads on looms in the 95 ordinary way.

3. Improvements in the treatment of the bast of the linden or lime-tree and willow 100 for the manufacture of webs, consisting in boiling the bast within an alkaline liquid, submitting the same to a second boiling process during 15-30 minutes within a closed vessel containing a 2%-3% liquid of soluble 105 glass, subdividing the softened bast into elementary fibrils, spinning threads from said fibrils mixed or combined with fibrils of another origin and using the threads for the manufacture of webs in the ordinary way. 110

4. Improvements in the treatment of the bast of linden or lime-tree and willow for the manufacture of webs, consisting in boiling the bast separated from the outer bark 5 within an alkaline liquid, cementing together the ends of the separate short bast films to form a long film, subdividing the latter into strips or flat threads, spooling the said strips or threads and, utilizing the flat 10 threads in combination with spun threads

for the manufacture of webs on ordinary looms in the usual manner.

In testimony that I claim the foregoing as my invention, I have signed my name in presence of two subscribing witnesses.

ALEXANDRE WAGANOFF.

Witnesses:

W. M. SEININGER,  
H. A. LOVIAGUINE.

Copies of this patent may be obtained for five cents each, by addressing the "Commissioner of Patents, Washington, D. C."